

June 8, 1948.

E. P. DAVEY ET AL

2,443,157

PHOTOGRAPHIC EMULSION CONTAINING BENZAL PYRUVIC ACID DERIVATIVES

Filed Jan. 9, 1946



SAME AS D+I GRAM PER LITER OF  
4-DIMETHYL-AMINOBENZAL  
PYRUVIC ACID



Edward Philip Davey  
Edward Bowes Knott  
Inventors

by *Newton A. Perkins*

R. Frank Smith  
Attorneys

## UNITED STATES PATENT OFFICE

2,443,157

PHOTOGRAPHIC EMULSION CONTAINING  
BENZAL PYRUVIC ACID DERIVATIVES

Edward Philip Davey and Edward Bowes Knott,  
Middlesex, England, assignors to Eastman  
Kodak Company, Rochester, N. Y., a corpora-  
tion of New Jersey

Application January 9, 1946, Serial No. 640,099  
In Great Britain February 9, 1945

6 Claims. (Cl. 95—7)

1

This invention relates to photographic materials, especially to sensitive silver salt emulsions and to methods of manufacturing such materials.

It is known to incorporate in photographic layers, substances which absorb some particular waveband of light, for instance, for some purposes a yellow dye is incorporated in a sensitive silver halide emulsion in order to absorb blue light and thereby reduce the gamma of the emulsion when exposed to blue light.

For some purposes it is desirable to incorporate in a photographic layer, a substance which absorbs ultra-violet light. To be of general use such a substance must satisfy various requirements. For instance, it is often desirable that it should be water soluble. If it is to be incorporated in a sensitive silver salt emulsion, for instance, a silver bromide, or chloride, or chloro-bromide emulsion, it should be such that it has little or no deleterious effect on the emulsion, for instance it should preferably have no effect on the emulsion sensitivity other than to reduce its gamma by absorbing light in the ultra-violet.

We have found that certain derivatives of pyruvic acid are especially useful for this purpose. The benzal pyruvic acids and their salts are especially valuable. Many of these substances absorb highly in the waveband 310 to 350  $\text{m}\mu$  but have little or no absorption in the visible light range.

It is, accordingly, an object of our invention to provide new photographic materials. A further object is to provide new methods for preparing such materials. Other objects will become apparent hereinafter.

In accordance with our invention there is provided a light-sensitive photographic element comprising a light-sensitive layer, said element including a layer containing an ultra-violet-light-absorbing amount of a compound having the formula



where R represents an aryl group and R' represents hydrogen or a halogen. Such compounds may advantageously be used in the form of their alkali metal salts, such as the sodium salts, or as their ammonium salts. The preferred compounds are the benzalpyruvic acids which often exist in two forms, one being colourless and the other having a yellowish tinge, and it is the latter form which are of value in the present invention.

2

In a particularly advantageous form of the present invention the compounds of the formula



are incorporated in the light-sensitive element with a compound of the type described in co-pending U. S. Patent 2,403,708, granted July 9, 1946, especially the nitranilines, or with the compounds described in application Serial No. 646,205, filed February 7, 1946, e. g. the nitraniline sulfonic acids.

Substances which can be used in the present invention are given in the following list which 15 gives also the literature references where their preparation is described (the abbreviation J. A. C. S. stands for the Journal of the American Chemistry Society). The position of maximum absorption is indicated in the last column; where 20 the substance stated is known to exist in two forms, it is the coloured form which is here referred to.

|     |                                                                         | Max $\text{m}\mu$ |
|-----|-------------------------------------------------------------------------|-------------------|
| 1.  | Benzal pyruvic acid, J. A. C. S. 1924, 46, 785                          | 300               |
| 2.  | 4-methylbenzal pyruvic acid, J. A. C. S. 1938, 60, 2469                 | ca. 300           |
| 3.  | 4-bromobenzal pyruvic acid, J. A. C. S. 1940, 62, 2515                  | ca. 300           |
| 4.  | $\beta$ -Bromo-4-bromobenzal pyruvic acid, J. A. C. S. 1940, 62, 2515   | 310               |
| 5.  | 4-methoxybenzal pyruvic acid, J. A. C. S. 1926, 48, 2459                | 330               |
| 6.  | $\beta$ -Bromo-4-methoxybenzal pyruvic acid, J. A. C. S. 1926, 48, 2459 | 335               |
| 7.  | 3-methoxybenzal pyruvic acid, J. A. C. S. 1933, 55, 4643                | 340               |
| 8.  | 2-methoxybenzal pyruvic acid, J. A. C. S. 1928, 50, 2807                | 345               |
| 9.  | 3:4-dimethoxybenzal pyruvic acid, J. A. C. S. 1935, 57, 211             | 345               |
| 10. | $\beta$ -Bromo-4-ethoxybenzal pyruvic acid, J. A. C. S. 1941, 63, 237   | 350               |
| 11. | 4-dimethylaminobenzal pyruvic acid                                      | 330               |

Compound No. 11 was prepared as follows: 35 p-dimethylaminobenzaldehyde (14.9 g.) and pyruvic acid (8.8 g.) were mixed at 5° C. and a 12.5% water-methanol (1:1) solution of potassium hydroxide (40 cc.) added. A yellow colour developed. Methyl alcohol (50 cc.) was added 40 and stirred till the solid had dissolved. After standing overnight the solution was diluted with water and acidified. Orange-yellow plates crystallised.

The effect of adding the above described substances to a gelatino-silver bromide emulsion is 45 illustrated by the examples described with reference to the accompanying drawings showing the gammas obtained at various wavelengths. The emulsion used contained in one litre, 50 50 grams of gelatin and an amount of silver bromide equivalent to 57 grams of  $\text{AgNO}_3$ . The substances chosen from the above given list were added in aqueous solution and in all cases the finished emulsion was coated at the rate equivalent 55 to 0.5 gram of  $\text{AgNO}_3$  per square foot. The

gamma values given in the drawings were measured in the manner given in Patent 2,403,708.

In Figure 1, curve A is for the emulsion without any additions. Curve 5 is for that emulsion containing 1.5 grams per litre of the sodium salt of the substance numbered 5 above; curves 6, 11 and 9 are likewise for the same emulsion as A but containing the same quantity of the sodium salt of the substances numbered 6, 11 and 9 respectively.

In Figure 2, curve B is for the same emulsion again as A but containing 1.0 gram per litre of p-nitraniline in alcohol (see Patent 2,403,708). Curve C is for the same emulsion as B but with the further addition of 1.0 gram per litre of the substance numbered 5 above. Curve D is for the same emulsion as A but containing 1.5 grams per litre of 1-amino-4-nitrobenzene-2-sodium sulphonate (see application Serial No. 646,205, filed February 7, 1946), and curve E is for the same emulsion as D but with the further addition of 1.0 gram per litre of the substance numbered 11 above.

What we claim as our invention and desire to be secured by Letters Patent of the United States is:

1. A light-sensitive photographic element comprising a support having thereon a silver halide emulsion layer containing an ultra-violet-light-absorbing amount of a benzal pyruvic acid.

2. A light-sensitive photographic element comprising a support having thereon a silver halide emulsion layer containing from 1 gram to 1.5 grams per liter of emulsion of a 4-methoxy benzal pyruvic acid.

3. A light-sensitive photographic element comprising a support having thereon a silver halide emulsion layer containing from 1 gram to 1.5 grams per liter of emulsion of  $\beta$ -bromo-4-methoxy benzal pyruvic acid.

4. A light-sensitive photographic element comprising a support having thereon a silver halide emulsion layer containing from 1 gram to 1.5 grams per liter of emulsion of 3,4-dimethoxy benzal pyruvic acid.

5. A light-sensitive photographic element comprising a silver halide emulsion layer containing an ultra-violet-light-absorbing amount of a compound selected from the class consisting of compounds having the formula:



15 where R represents an aryl group and R' is selected from the class consisting of hydrogen and halogen, and the alkali metal and ammonium salts of said compounds.

6. A light-sensitive photographic element comprising a support having thereon a silver halide emulsion layer containing from 1 gram to 1.5 grams per liter of emulsion of the sodium salt of a benzal pyruvic acid.

EDWARD PHILIP DAVEY.  
EDWARD BOWES KNOTT.

#### REFERENCES CITED

The following references are of record in the file of this patent:

#### UNITED STATES PATENTS

| Number       | Name                 | Date         |
|--------------|----------------------|--------------|
| 35 2,241,289 | Carroll et al. _____ | May 6, 1941  |
| 2,403,708    | Davey et al. _____   | July 9, 1946 |

#### FOREIGN PATENTS

| Number     | Country             | Date         |
|------------|---------------------|--------------|
| 40 524,377 | Great Britain _____ | Aug. 5, 1940 |